

## UNITED STATES PATENT OFFICE.

LESTER KIRSCHBRAUN, OF CHICAGO, ILLINOIS.

## BITUMINOUS COMPOSITION.

No Drawing.

Application filed April 25, 1924. Serial No. 708,887.

This invention relates to a process and product of forming a non-fluid or non-fusible bituminous binder or composition.

In the particular embodiment of this invention the product desired to be produced results from the emulsification of a fusible bituminous binder with bentonite or analogous, argilliferous substances in an aqueous vehicle and the subsequent removal of the aqueous medium without agitation.

This application is in part an improvement of co-pending application filed by me; Serial #463,945, April 23rd, 1921.

One process by which this product may be formed is described in the above referred to application and in order to produce the result desired requires only the predetermination of the quantity and character of bentonite or analogous argillaceous emulsifying agent or agents used in forming the emulsion.

It should be understood that the desired product comprises only the water-free residue of the process above referred to with such modifications of content of bentonite or analogous agent or agents as are required to bring about the desired result.

I have found that in carrying out the above process if a quantity of bentonite is used which is in excess of one-tenth of the amount of asphalt emulsified that the resulting product when allowed to dry without disturbance, produces a bituminous composition which is apparently homogeneous, adhesive, waterproof, and possesses considerable ductility. In actual practice, it has been found advantageous to employ considerably less than thirty per cent, and not more than forty per cent, of bentonite relative to the asphalt emulsified. It is characterized by its ability to resist heat without flowing or becoming liquid. If a sheet or relatively thick film of this material, (say  $1/4$ "- $1/2$ " thick) which has been spread and dried on a metal surface be subjected while in an inclined position to the action of intense heat on the surface thereof (as from a Bunsen burner) the bituminous composition described will not flow or run as would be the case with the original asphalt used, but would retain its position without exhibiting any indications of fluidity. When the composition has been subjected to sufficient heat to drive off volatile constituents, these volatile constituents may take fire and the mass may become destroyed by the removal of

the volatile matter, without change of shape or structure.

This property of the bituminous material described above is of value in connection with roofing or waterproofing wherein the bituminous material may be applied to inclined surfaces or vertical walls or to stacks which are highly heated and to like structures requiring protection against heat, corrosion or the action of the elements.

It is evident that the peculiar property as developed by this bituminous composition is a result of its having undergone emulsification and in particular the character and the amount of bentonite or other emulsifying agent or agents used appears to be a controlling factor in regulating the infusibility of the end product.

While I am not able to explain completely all the changes involved in this phenomena, it appears likely that while the material is in an emulsified form, the dispersed particles of bituminous material carry adsorbed films of bentonite or similar agent or agents upon their surfaces and that upon the removal of the water without agitation, these films remain in place preserving a film or honeycomb structure in the coalesced end product. If these films above referred to are sufficiently strong and durable to persist in the coalesced end product, the end product possesses the characteristics of a gel, thereby losing its ability to fuse and become fluid under the action of heat. This is strongly indicated by the fact that the same bituminous emulsion which will produce a non-fusible end product in the absence of agitation (after removal of water) will, if agitated or disturbed, produce a fusible end product, indicating the effect of agitation in breaking up the gel or honeycomb structure produced by the emulsifying agent or agents.

It will be understood then, that in applying this composition in a practical way, as for instance, to a vertical, concrete wall for waterproofing purposes, the emulsified material will be spread over the wall as a heavy plaster and allowed to dry out by natural means, and without agitation or disturbance of the coating thus formed, either during the drying operation or after the material has become set. In this way, the infusible character of the plastic will be preserved and the product will possess the characteristics described above.

Luminous material of wide variety can be converted to this form almost regardless of the melting point of the original material. That is, it is possible to use asphalt or tar or animal or vegetable pitch having, say, a melting point of 110 degrees F. and by emulsifying with bentonite or analogous emulsifying agent or agents in excess of one-tenth by weight of the latter relative to binder, the resulting product when dried out will be infusible and will have lost its melting point. Even more or less liquid hydrocarbons, as for instance, heavy petroleum residuum, may be converted to this infusible form by use of the requisite quantity of bentonite or similar emulsifying agent or agents.

The process may be carried out in accordance with the disclosure of said co-pending application which briefly may be as follows:

An aqueous paste may be formed of bentonite and water. A single bentonite may be used by itself or there may be employed a combination of bentonites with clays having varying properties, or a combination of bentonites with other emulsifying materials, either argilliferous or otherwise.

This aqueous paste is preferably brought to about the temperature of the melting point of the bituminous material which is to be emulsified. The bituminous material, in liquid condition, and at a temperature of approximately 100 deg. above its melting point, may be slowly added to the aqueous paste with thorough agitation so as to produce dispersion of the bituminous material.

Water may be added from time to time as the batch thickens in order to maintain a desired viscosity in the batch, as well as a regulated temperature, while further additions of bitumen are being made.

When the desired amount of bitumen relative to the emulsifying agent has been incorporated, the batch is completed and the pasty mass is ready for use.

It should be understood that the proportions of bentonite to asphalt indicated above will be varied with the character of the bentonite and the character of the bituminous material, the amount of the latter being always such as to produce in the end product the characteristic infusibility referred to above.

Generally, the greater the viscosity of an aqueous solution of a given concentration of the bentonite or argillaceous mixture, the less of the material is required to produce the desired result.

I am aware that heretofore, compositions have been produced in which emulsifying agents of varying properties have been employed, but I believe I am the first to discover that by regulating or controlling the quantity and the character of the emulsifying agents employed, the character of the resulting product can be accurately controlled and a product produced which is within a range of fusibility or nonfusibility which latter feature can be pre-determined.

I claim as my invention:

1. An infusible composition comprising a major portion of a normally fusible bitumen pitch type base, and a minor portion of an emulsifying agent having substantially the functions of bentonite, said composition possessing a gel or honeycomb-like structure of such stability as to withstand flow under heat substantially above the melting point of the base.

2. An infusible composition comprising a major portion of a normally fusible bitumen pitch type base, and a minor portion of bentonite, said composition possessing a gel or honeycomb-like structure of such stability as to withstand flow under heat.

3. An infusible composition comprising a major portion of a normally fusible bitumen pitch type base, and a minor portion, substantially ten per cent, of bentonite, said composition possessing a gel or honeycomb-like structure of such stability as to withstand flow under heat substantially above the melting point of the base.

4. An infusible composition comprising a major portion of a normally fusible bitumen pitch type base, and a minor portion of bentonite-like material, the bitumen present greatly predominating relative to the amount of bentonite-like material, said composition possessing a gel or honeycomb-like structure of such stability as to withstand flow under any heat conditions.

5. An infusible bituminous composition derived from an emulsion of bitumen and a material possessing substantially the functions of bentonite, the amount of bitumen present in the composition greatly exceeding that of the bentonite-like material, the said composition being characterized by a small portion of the bentonite-like material relative to the bitumen present, and the ability of the composition to withstand flowing to the point of decomposition temperature of the bitumen.

LESTER KIRSCHBRAUN.